

Feb. 26, 1946.

J. HEUBERGER

2,395,408

METHOD OF MAKING GRAPHITE MOLDS

Filed April 2, 1942



Fig. 1

Fig. 2

INVENTOR

*Josef Heuberger*

By *G. F. Ondurth*

ATTORNEY

## UNITED STATES PATENT OFFICE

2,395,408

## METHOD OF MAKING GRAPHITE MOLDS

Josef Heuberger, Stockholm, Sweden, assignor to  
 Aktiebolaget Hammarbylampan, Stockholm,  
 Sweden, a company of Sweden

Application April 2, 1942, Serial No. 437,445  
 In Sweden February 15, 1941

2 Claims. (Cl. 18—55)

The present invention relates to a method of making molds from graphite. In the metal-ceramic scopes of activity, there is a need for molds from heat resistive material. For this purpose graphite has found a very extensive use. Hitherto, hollow molds of the "cup type" closed at the bottom generally are manufactured by turning, grinding or some other working involving the detachment of chips. Disregarding the loss of material, this manufacture is tedious and does not enable obtaining surfaces as smooth as desirable. Moreover, the surfaces operated upon are rendered rather porous, so that the products made in the molds will obtain a rather irregular surface structure. Endeavours have been made, therefore, to press such molds from graphite powder or from mixtures of graphite and carbon powder with binding agents, and then to undertake sintering of the molds, that is to say, a method analogous to the manufacture of carbon electrodes, carbon brushes or the like.

However, due to the fact that these graphite molds are to be pressed as hollow bodies having a bottom, the ordinary powder pressing technique cannot be applied for the reason that the distribution of pressure within the powder mass becomes too irregular. This is so because if graphite powder or a powder mixture with appreciable contents of graphite be subjected to pressure, the graphite particles will orient themselves (occupy a determined direction) relatively to the direction of pressure on account of their pronounced leaf-like structure, so that the powder will "flow," preferably in a direction influenced by the graphite leaves or flakes. This flow of material along the gliding surfaces referred to will then cause initiations of rupture in the pressed body, which are frequently so pronounced that the body cannot be removed from its press mold, without cracks being produced.

According to the present invention, a method has been evolved which solves this problem and eliminates the difficulties by the graphite powder mass being pressed in a manner such that the pressure in the powder mass will be the same all over in planes at right angles to the direction of compression. Hereby the advantage is attained that lateral creeping does not occur, so that the powder particles, disregarding the reduction of distance in the direction of pressure, will maintain their proper mutual positions. According to the invention, this is attained, for instance, by making the stamp as a divided body, and by adapting the pressure on the various parts of the stamp, so that those portions of the powder

mass which are actuated by the pressure will show the same degree of compression at every moment of the pressing operation.

On the accompanying sheet of drawings:

Fig. 1 is a diagrammatic representation of one embodiment of the invention;

Fig. 2 shows a modified form of bottom piece.

In order properly to adapt the pressure on the various parts of the stamp, the same powder as that from which the mold body is manufactured may be used as a pressure-regulating material. Such a method is illustrated in Figure 1. A stamp consisting of an external member, and provided with a top plate 8, is filled internally with graphite powder 9. The stamp operates in a matrix 10 provided with a bottom plate 11. If at the commencement of the pressing operation the height of the quantity of powder enclosed within the stamp is designated by A and the height of the quantity of powder between the inner stamp member 7 and the bottom plate 11 is denoted by B, and the height between the outer stamp member 6 and the said plate 11 is designated by C, and the height is so adapted that  $A+B=C$ , then the condition for the obviation of creepings is fulfilled, that is to say, the graphite will be compressed at the same time in every part of the press body, and there will be an equal pressure in planes extending at right angles to the direction of pressure. In applying this method excellent results are obtained. Due regard must be paid, however, to the fact that an additional press body will be formed from the powder quantity 9 in every pressing operation.

According to the method described above, the problem has been solved by the use of a divided stamp. However, the conditions referred to in connection with the stamp apply in regard to the bottom piece too. In an analogous manner also this bottom piece may be composed of mutually movable parts, the movement of which, taking place under the action of pressure, is controlled by filling the body with pressing mass or by the use of springs.

In the examples above referred to, the methods relate primarily to the manufacture of a graphite cup, wherein the distribution of pressure in the pressing mass can be readily anticipated on account of the simple geometry of the press body. On the other hand, if graphite molds of more complicated outlines are to be pressed, it is difficult and often practically impossible to form an idea as to the distribution of pressure in the graphite mass. Without a knowledge of the pressure distribution it is impossible to construct the

tool for pressing the graphite body so that the movable parts of the stamp or bottom piece will obtain the proper shape. The flow at the compression is dependent not only on the inner friction, but also on the friction against the walls of the tool (the press chamber), and with complicated shapes this factor cannot be calculated in a simple and practicable manner.

Another difficulty in calculating the distribution of pressure in the pressing mass may reside in the composition of the mass proper. As long as pure graphite powder is operated with, one knows rather well the internal friction and the manner in which the individual graphite particles will be directed on account of their leaf-like structure, the planes of the flakes turning into a position so as to lie at right angles to the direction of pressure; the pressing mass is non-isotropic as regards pressure. In order to obtain greater strength or other desirable properties, such as hardness, porosity of the molded body after the pressing operation and/or upon sintering, it is frequently necessary, however, to mix the graphite with other more or less plastic substances adapted to bind at the sintering or pressing operation in accordance with the effect desired. Such additional substances are carbon, coke, soot, for example, or syrup-like solutions, with which the powder is impregnated, without losing its pulverulent nature at pressing temperature, if desired after special drying. Inasmuch as these additional substances generally do not have a leaf-like structure, the said admixture will cause the pressing mass to lose some of its property of being non-isotropic as regards pressure.

The properties of flow of the pressing mass will be substantially altered, and the calculation of the distribution of pressure in the mass during compression is rendered particularly difficult, if the substances to be admixed are of such a nature that their plastic properties are changed through the heating caused by the friction when the mass is compressed. This difficulty is obviated according to another method in accordance with the invention by using plastic parts in the stamp or bottom piece of the tool. If, in performing the pressing operation, a sufficiently plastic bottom piece 11a is used, such bottom piece will, upon one or more pressing operations, take the shape shown in Figure 2, that is to say, the bottom piece has adapted its shape according to the distribution of pressure so that its surface facing the pressing chamber constitutes the geometric locus for equal pressures. The bottom piece thus molded may therefore be used directly for subsequent pressing operations to enable obtaining graphite molds without any rupture initiations caused by an irregular pressure distribution, or, one may use the shaped plastic bottom piece as a pattern for the manufacture of a bottom piece from a more permanent material. As a plastic material, porous press bodies will be found particularly suitable, but also sintered press bodies of metal powder from soft ductile metals such as copper, to which the graphite body does not adhere, will be found useful. When lower pressures are operated with, obviously such elastic substances as rubber will adopt a pressure-equalizing shape which is re-

stored into the original shape after the pressing operation.

As many changes could be made in the above method and construction and many apparently 5 widely different embodiments of the invention could be made without departing from the scope thereof, as defined by the following claims, it is intended that all matter contained in the above 10 description shall be interpreted as illustrative and not in a limiting sense.

What I claim is:

1. A method of producing essentially cup-like articles from pulverulent material such as graphite, which comprises confining the said material 15 in a pressure mold having a bottom piece, between the said bottom piece and a vertically disposed pressure applicator longitudinally movable in the mold, said applicator comprising at least two relatively longitudinally movable pressure-applying 20 parts, the lower ends of which terminate in vertically spaced horizontal planes, which parts, during the compressing operation act in the same direction longitudinally of the said parts and of said mold, said pressure applying parts also defining a completely closed space therebetween confining a pulverulent material having substantially the same compressibility as said first-named pulverulent material in the space between the relatively movable parts of the pressure 25 applicator, the said materials being under the same state of compression initially and the initial height of the said first-named pulverulent material when the mold is full and the material is in the un- 30 compressed state being substantially equal to the sum of the initial height of the pulverulent material between the said applicator parts and the initial distance between the bottom of the lowermost of the said parts and the bottom piece of the mold, and then applying pressure to said first-named pulverulent material through the said applicator parts and the material comprised therebetween, whereby a substantially equal pressure is maintained throughout the material being 35 compressed in planes at right angles to the direction of compression.

2. In apparatus for producing essentially cup-like articles from compressible material, a pressure mold having a bottom piece, a pressure applicator longitudinally movable in said pressure mold, said pressure applicator comprising at least two relatively longitudinally movable pressure-applying parts, the lower ends of which terminate in vertically spaced horizontal planes, which parts, during the compression operation act in the same direction longitudinally of the said parts and of the said mold, said pressure-applying parts defining a recess therebetween, said recess being filled with pulverulent material of substantially the same compressibility as said first-named compressible material, the longitudinal extent of said recess when the mold is full and said compressible material is in uncompressed state being substantially equal to the difference between the distances from the several lower ends of said pressure-applying parts to said bottom piece.

JOSEF HEUBERGER.